

## UNITED STATES PATENT OFFICE

GEORGE ALLEN OSTERDAY, OF HAMILTON, OHIO, ASSIGNEE OF ONE-HALF TO EDWARD DOME, OF COLLINSVILLE, OHIO

## COMPOSITE ROOFING COMPOUND

No Drawing.

Application filed April 25, 1928. Serial No. 272,865.

This invention relates to an improved composite roofing compound to be used as a covering for either old or new roofs, and it has reference to the character of compound, which is mixed hot for ready application to the roof, after which it may be rolled to press it tightly into the pores of the roof.

Briefly stated, the purpose of the compound is to provide a moderate priced roof whose properties permit the production of a product possessing durability, lightness in weight, insulation and shelter properties, and other features not found in similar roofing compounds.

The compound is applicable to roofs of wood, or metal, or to old composite surfaces.

The preferred formula for the average pitched roof is as follows:

|                              | Per cent |
|------------------------------|----------|
| Pitch—M. P. 285 to 300       | 40       |
| Trinidad lake asphalt cement | 40       |
| Ground cork                  | 15       |
| Ground asbestos              | 5        |
|                              | 100      |

I also propose the following variation in mix, to meet the needs of different pitched roofs which are exposed to the sun. This mixture is as follows:

|          | Per cent |
|----------|----------|
| Pitch    | 25 to 40 |
| Asphalt  | 25 to 50 |
| Cork     | 35 to 40 |
| Asbestos | 5 to 10  |

Obviously, the asphalt is employed for its long life, durability, viscosity, strength, and resistance to the elements.

Pitch is employed in the mixture to harden and preserve the asphalt.

Cork is employed as a filler and because of its ability to yield and accommodate contraction and expansion, of the compound.

Asbestos serves as a binder and heat resister.

In applying the compound, it is advisable to first use a priming coat of material which is preferably composed of 70% of asphalt, mixed with 30% common oil. In applying the compound, it must be put on the roof hot. It is then smoothed off, with a hot towel, then rolled with a hot roller which presses the mix-

ture tightly in the pores, crevices, and irregularities.

The mixture adheres to metal, cement or wood, and can be put on old or new roofs without requiring unusual skill.

It will be observed that there are no nails, no trimming or fitting of gutters and valleys. Consequently, the compound is applied in little time and with ease. When finished it has a smooth surface and leaves no sand to wash into gutters to clog the flow of water or to rust the gutter.

It is one solid sheet without a seam or a joint in it. Hence, it prevents leaks and reduces fire hazard. It has the desired resistance to wind and hail, and possesses other advantages which permit it to fulfill the requirements of a compound of this class.

Changes in proportion, and ingredients may be resorted to within the scope of the adjoining claim.

Having thus described my invention, what I claim as new is:

A roofing compound comprising a mixture of pitch 25 to 40%, asphalt 25 to 50%, cork 35 to 40% and asbestos 5 to 10%.

In testimony whereof I affix my signature.

GEORGE ALLEN OSTERDAY.

55

60

65

70

75

80

85

90

95

100